

## UNITED STATES PATENT OFFICE

2,104,694

## WELDROD

Anthony G. de Golyer, New York, N. Y., assignor  
to Vulcan Alloy Corporation, a corporation of  
Delaware

No Drawing. Application March 12, 1937,  
Serial No. 130,494

1 Claim. (Cl. 219—8)

This invention relates to a new alloy steel and relates particularly to an alloy steel containing manganese and boron, as well as certain other elements in the form of a weld rod for the production of welded surfaces or sections characterized by a relatively high degree of hardness, resistance to abrasion and resistance to deformation under impact.

This application is a continuation in part of 10 my co-pending application Serial No. 96,463, filed August 17, 1936.

In many industrial applications it is desirable to apply a facing or inlay of hard, wear resistant metal to parts of machinery or other equipment 15 exposed to abrasion or impact. Various alloys and materials have been proposed for this purpose. All of such heretofore suggested compositions contain high percentages of alloy elements, together with at least approximately 1% or more 20 carbon. In general, weld metal deposited with such compositions may have relatively high hardness but all of such deposits are comparatively brittle and consequently are not suitable for use on surfaces exposed to impact or shock.

The object of the present invention is to provide 25 an alloy which may be readily deposited by fusion welding, and which produces weld metal having relatively high strength, high resistance to deformation under impact and relatively high 30 hardness.

I have found that an alloy composed of manganese 1% to 6%, boron 0.25% to 2.50%, nickel 0.50% to 5%, carbon 0.10% to 0.60% and the balance principally iron possesses high hardness, 35 high strength and is extremely resistant to deformation under impact when deposited by means of welding. Metal so deposited has a hardness of from 350 to approximately 500 Brinell depending, in part, on the composition 40 of the base metal and the ratio of dilution. Weld deposits of the alloy which have been subjected to an appreciable amount of cold work or impact usually show an increase in hardness of from 50 to 150 Brinell numbers.

A distinct advantage of the present alloy is 45 that it may be readily welded on steel of any carbon content, 14% manganese steel, rail steel and virtually all types of alloy steels. The com-

bination of physical properties and characteristics possessed by this alloy render it particularly valuable for facing new or worn rail ends, new or worn railroad track equipment, such as frogs, crossovers, switch points, etc., for repairing or refacing manganese steel and other alloy steels and for facing wearing surfaces of carbon steels. Weld deposits of this alloy are characterized by an appreciably greater hardness than weld deposits of heretofore known manganese steel, 10 and are further characterized by materially greater resistance to deformation under impact than any of the heretofore known manganese steels.

The essential components of my alloy are manganese, boron, nickel, carbon and iron. The principal constituent of the alloy is iron. The manganese content should be between 1% and 6%, the boron content between 0.25% and 2.50%, the nickel content should be between 0.50% and 5% and the carbon content should not exceed approximately 0.60%; the balance being substantially iron. It will be understood that the alloy will usually contain minor amounts of phosphorous, sulphur and other impurities incidental to manufacture; the amounts of such impurities should be within the maximum limits ordinarily prescribed for alloy steels.

As specific examples of alloys within the scope 30 of the present invention, which I have found to be suitable for facing by welding of new or worn equipment, are the following: Manganese 1.80%, boron 0.35%, nickel 1.50%, carbon 0.20% and the balance substantially iron; manganese 4.60%, boron 1.10%, nickel 2.50%, carbon 0.40% and 35 the balance substantially iron; manganese 5.50%, boron 1.30%, nickel 3%, carbon 0.25% and the balance substantially iron.

It will be understood that minor amounts of silicon will usually be present in the alloy incidental to manufacture. The silicon content should not exceed approximately 1%.

I claim:

A weld rod comprising a metallic composition 45 containing manganese 1% to 6%, boron 0.25% to 2.50%, nickel 0.50% to 5%, carbon up to a maximum of 0.60% and the balance substantially iron.

ANTHONY G. DE GOLYER.